

Patented July 15, 1924.

1,501,183

# UNITED STATES PATENT OFFICE.

NAPOLEON PETINOT, OF NEW YORK, N. Y.

## METHOD OF MAKING CHROMIUM STEEL AND CHROMIUM IRON.

No Drawing.

Application filed July 18, 1922. Serial No. 575,804.

To all whom it may concern:

Be it known that I, NAPOLEON PETINOT, a citizen of the United States of America, and a resident of the city, county, and State 5 of New York, have invented new and useful Methods of Making Chromium Steel and Chromium Iron, of which the following is a full, clear, and exact description.

This invention relates to a new method of 10 making additions of chromium to steel or iron.

In a co-pending patent application Serial 15 No. 575,803, filed July 18, 1922, I have described my new alloy composed of chromium, iron, and silicon and a method of making the same. In this application, I disclose a method of using such alloy in the manufacture of chromium steel or chromium iron.

In making chromium steels the common 20 practice of the art has been first to prepare a bath of molten steel. Then by suitable treatment the bath is adjusted until it has the desired composition, as regards the usual components of ordinary steels such as iron, carbon, silicon, manganese, sulphur, and phosphorus. Then, as the last step, towards the end of the heat and before the furnace is tapped, a ferro-chromium alloy is added in such quantity that the desired content of 25 chromium will be found in the finished steel. Frequently it is found necessary at this last stage to add some silicon to the steel in order that it may contain the amount of that metal that is called for in the specifications for the 30 finished product. If silicon is thus employed, its introduction is made in the ladle when the furnace is tapped.

One of the most serious difficulties encountered in the manufacture of chromium 35 steels by this method is that a large amount of chromium is lost by oxidation when the ferro-chromium is added to the bath. This difficulty makes the accurate adjustment of the chromium content a very difficult and delicate thing. Moreover, this method is expensive since the oxidized chromium is slagged off, and chromium is an expensive 45 element.

A typical analysis of ferro-chromium, 50 such as is used in making chromium steels, (I refer particularly to those grades which have a carbon content of 8% or less) is as follows:

Cr. 64.0%; Fe. 28.5%; C. 5.5%; Si. 0.4%; 55 Al. 0.5%; Mn. 0.15%; Ca. 0.25%; S. 0.04%; P. 0.03%.

It will be observed that the carbon content of this ferro-chromium amounts to 5.5%. When such an alloy is added to the steel bath, it is recognized that the carbon, to a certain extent, prevents the loss of chromium by oxidation, so that the higher the percentage of carbon present, the less will be the chromium loss.

This, however, is not a satisfactory method of taking care of the chromium losses due to oxidation, since some of the carbon is apt to be taken up by the steel thereby disturbing the desired carbon content of the finished product. On the other hand, the lower the carbon content is in the added ferro-chromium the more costly the ferro-chromium is and hence the more serious economically, is the loss of chromium by oxidation.

It should also be noted that the typical commercial grades of ferro-chromium are always low in silicon; the silicon content usually running as low as 0.4 to 1.5 per cent.

The invention described herein improves 80 the methods heretofore used in that the loss of chromium by oxidation is substantially eliminated.

In carrying out my invention, I prepare my steel or iron in the furnace (for example, 85 an open hearth furnace) in the usual way. Just before tapping the furnace I add a quantity of my ferro-chromium-silicon alloy, which usually and preferably contains from two per cent to ten per cent of silicon. The amount of such alloy to be added depends upon the amount of chromium which is desired in the finished product.

Usually the ferro-chromium-silicon alloy used in carrying out my process has a silicon 95 content of from two to ten per cent, that content being sufficient to protect the chromium from oxidation without affecting the silicon content of the bath.

My invention, however, is not confined to 100 the addition of a ferro-chromium-silicon alloy of such low silicon content as that last above described. I have found that an alloy of such character may be advantageously used which has as high a silicon content as 105 fifty per cent when it is desired to produce a chromium steel of high silicon content.

In carrying out my invention, I may employ a ferro-chromium-silicon alloy having such a silicon content that the silicon not 110 only protects the chromium from oxidation, but also leaves a residuum of silicon in the

bath thereby increasing the absolute quantity of silicon in the bath.

Obviously some modifications of my invention as herein described may be made without departing from the spirit thereof, and I do not wish to be limited to the exact method in all of its details as herein described.

Having thus described my invention, what I claim is:

1. A method of making chromium steel or chromium iron comprising the addition to the molten iron bath of a ferro-chromium-silicon alloy containing sufficient silicon to protect the chromium from oxidation.

2. A method of making chromium steel or chromium iron comprising the addition to the molten iron bath of a ferro-chromium-silicon alloy containing sufficient silicon to not only protect the chromium from oxidation but also to bring the silicon content of the finished product up to the desired amount.

3. A method for making chromium steel or chromium iron comprising the addition to the molten iron bath of a ferro-chromium-

silicon alloy containing sufficient silicon to not only protect the chromium from oxidation but also to bring the silicon content of the finished product up to at least two and one-half per cent of silicon.

4. A method for making chromium steel or chromium iron comprising the addition to the molten iron bath of a ferro-chromium-silicon alloy containing sufficient silicon to not only protect the chromium from oxidation but also to bring the silicon content of the finished product up to not more than fifty per cent of silicon.

5. A method for making chromium steel or chromium iron comprising the addition to the molten iron bath of a ferro-chromium-silicon alloy containing sufficient silicon to not only protect the chromium from oxidation but also to bring the silicon content of the finished product up to not less than two and one-half per cent and not more than fifty per cent of silicon.

In witness whereof, I have hereunto signed my name.

NAPOLEON PETINOT.